

2,950,250

**SILICONE LUBRICATING OIL COMPOSITION  
CONTAINING ESTER FOR IMPROVED LU-  
BRICITY AND THERMAL STABILITY**

Morton Z. Fainman, Chicago, Ill., assignor to Standard Oil Company, Chicago, Ill., a corporation of Indiana

No Drawing. Filed Feb. 29, 1956, Ser. No. 568,436

5 Claims. (Cl. 252—49.6)

This invention relates to improvements in synthetic lubricant compositions and more particularly relates to improved silicone polymer lubricants having improved lubricity properties and good thermal stability.

Silicone oils used as lubricants possess good thermal stability and have a favorable viscosity-temperature relation or viscosity index (V.I.). They also possess desirable high flash point and low pour point characteristics. However, the silicone oils have poor lubricity properties which make them poor lubricants under boundary lubricating conditions, particularly for ferrous metal bearing surfaces. As a corollary to the poor lubricity, the silicones permit excessive wear.

It is an object of this invention to provide a silicone lubricant having improved lubricity properties. Another object of the invention is to provide a silicone lubricating oil composition having thermal stability, a high viscosity index and improved lubricity characteristics. Other objects and advantages of the invention will become apparent from the following description thereof.

In accordance with the herein-described invention, the foregoing objects can be attained by incorporating in silicone oil lubricants from about 5% to about 75%, and preferably from about 10% to about 45% of an ester of a straight chain aliphatic carboxylic acid of from about 4 to about 18 carbon atoms and a polyhydric alcohol free of beta hydrogen; that is, containing no hydrogen on the beta carbon atom. Illustrative of such esters are those having the general formula:



in which R and R' are the same or different straight chain alkyl radicals of from 4 to about 18 carbon atoms, R<sub>1</sub> and R<sub>4</sub> are selected from the group consisting of hydrogen, or alkyl radicals of from 1 to 4 carbon atoms and mixtures thereof, R<sub>2</sub> is selected from the group consisting of an alkyl radical of 1 to 6 carbon atoms, or a hydroxy methyl radical, and R<sub>3</sub> is selected from the group consisting of an alkyl radical of 2 to about 12 carbon atoms or a hydroxy methyl radical. The R<sub>2</sub> and R<sub>3</sub> groups may be the same or different.

Polyhydric alcohols free of beta hydrogen can be readily prepared to give a structure derived from neopentane. Acetaldehyde is treated with 5 equivalents of formaldehyde in an aqueous solution of calcium hydroxide at 15–45° to give pentaerythritol according to the following steps:



By choosing a different aldehyde or ketone as starting

material, we obtain other polyhydric alcohols. Illustrative of such polyhydric alcohols free of beta hydrogen are:



Examples of straight chain alkyl carboxylic acids with which polyhydric alcohols of the above type may be esterified are n-butrylic acid, n-pentanoic acid, n-octanoic acid, n-nonanoic acid (pelargonic acid), n-decanoic acid (capric acid), lauric acid, myristic acid, stearic acid, etc.

The esters of straight chain alkyl carboxylic acids and polyhydric alcohols free of beta hydrogens possess high viscosity index, high flash point, and good thermal stability characteristics as compared to the esters of branched chain acids. The differences in these physical properties between the esters of straight chain acids and the esters of branched chain acids are illustrated by the data in Table I.

TABLE I

| Acid b             | Pour Point, °F.  | Flash Point, °F. | Viscosity, Cs. |         | Viscosity Index |
|--------------------|------------------|------------------|----------------|---------|-----------------|
|                    |                  |                  | 100° F.        | 210° F. |                 |
| NEOPENTYL GLYCOL   |                  |                  |                |         |                 |
| n-C <sub>4</sub>   | -5               | 410              | 9.12           | 2.62    | 136             |
| n-C <sub>10</sub>  | -5               | 435              | 11.3           | 3.01    | 141             |
| n-C <sub>14</sub>  | <sup>a</sup> 93  |                  |                |         |                 |
| br-C <sub>8</sub>  | <-65             | 385              | 9.20           | 2.80    | 152             |
| br-C <sub>9</sub>  | <-65             | 380              | 14.0           | 3.07    | 78              |
| br-C <sub>10</sub> | <-65             | 395              | 15.2           | 3.19    | 73              |
| br-C <sub>13</sub> | -65              | 460              | 35.0           | 5.28    | 88              |
| TRIMETHYLOLETHANE  |                  |                  |                |         |                 |
| n-C <sub>8</sub>   | +35              | 535              | 21.0           | 4.48    | 147             |
| n-C <sub>10</sub>  | +5               | 535              | 24.5           | 5.12    | 150             |
| n-C <sub>14</sub>  | <sup>a</sup> 115 |                  |                |         |                 |
| br-C <sub>7</sub>  | -85              | 480              | 27.1           | 4.72    | 103             |
| br-C <sub>9</sub>  | -55              | 465              | 54.9           | 6.85    | 85              |
| br-C <sub>10</sub> | -55              | 510              | 46.5           | 6.42    | 95              |
| br-C <sub>13</sub> | -45              | 545              | 111.0          | 10.41   | 80              |
| TRIMETHYLOLPROPANE |                  |                  |                |         |                 |
| n-C <sub>8</sub>   | <-80             | 470              | 12.5           | 3.06    | 115             |
| n-C <sub>7</sub>   | <-80             | 495              | 15.2           | 3.51    | 125             |
| n-C <sub>8</sub>   | -65              | 505              | 19.0           | 4.09    | 135             |
| n-C <sub>9</sub>   | -55              | 525              | 22.9           | 4.62    | 135             |
| n-C <sub>10</sub>  | -20              | 540              | 27.6           | 5.42    | 142             |
| n-C <sub>14</sub>  | <sup>a</sup> 107 |                  |                |         |                 |
| br-C <sub>8</sub>  | -65              | 460              | 31.9           | 5.07    | 92              |
| br-C <sub>9</sub>  | -40              | 445              | 59.7           | 7.30    | 88              |
| br-C <sub>10</sub> | -60              | 530              | 50.8           | 6.80    | 95              |
| br-C <sub>13</sub> | -35              | 535              | 117.5          | 10.94   | 82              |

Footnotes at end of table.

| Acid b                          | Pour Point, °F. | Flash Point, °F. | Viscosity, Cs. |         | Viscosity Index |
|---------------------------------|-----------------|------------------|----------------|---------|-----------------|
|                                 |                 |                  | 100° F.        | 210° F. |                 |
| PENTAERYTHRITOL                 |                 |                  |                |         |                 |
| n-C <sub>6</sub>                | +30             | 555              | 34.7           | 6.23    | 135             |
| br-C <sub>6</sub>               | -60             | 495              | 55.6           | 7.39    | 102             |
| br-C <sub>8</sub>               | -30             | 505              | 129.2          | 11.60   | 82              |
| br-C <sub>10</sub>              | -45             | 520              | 92.1           | 9.85    | 93              |
| 2-BUTYL-2-ETHYL-1,3-PROPANEDIOL |                 |                  |                |         |                 |
| n-C <sub>9</sub>                | <-80            | 450              | 14.4           | 3.34    | 121             |
| n-C <sub>14</sub>               | +30             | 540              | 30.2           | 5.92    | 146             |
| n-C <sub>18</sub>               | +70             | 575              | 45.0           | 8.06    | 142             |

a Melting point, °F.

b n=straight chain acids.

br=branched chain acids.

In addition to the above physical properties, the esters of the straight chain acids possess better lubricity characteristics than do the esters of the branched chain acids. This is demonstrated by the data in Table II. The static ( $\mu_s$ ) coefficient of friction and the kinetic ( $\mu_k$ ) coefficient of friction were obtained on "stick-slip" machine described in the article by M. E. Merchant on "Characteristics of Typical Polar and Non-Polar Lubricant Additives Under Stick-Slip Conditions" in Lubrication Engineering, June 2, 1946, pp. 56-61. The described apparatus provides a means for determining the kinetic friction ( $\mu_k$ ) and the static friction ( $\mu_s$ ) between two metal surfaces and thereby a measure of the lubricity of the lubricant under boundary lubrication conditions. Smooth sliding, indicative of good lubricity, occurs when  $\mu_s/\mu_k$  is equal to or less than 1. When the value of  $\mu_s/\mu_k$  is greater than 1, sticking occurs.

TABLE II  
Boundary lubrication properties of polyhydric-alcohol esters

## COEFFICIENT OF FRICTION

| Acid               | Static, $\mu_s$ | Kinetic, $\mu_k$ | $\mu_s/\mu_k$ |
|--------------------|-----------------|------------------|---------------|
| NEOPENTYL GLYCOL   |                 |                  |               |
| n-C <sub>6</sub>   | 0.131           | 0.142            | 0.92          |
| n-C <sub>10</sub>  | 0.120           | 0.137            | 0.88          |
| br-C <sub>6</sub>  | 0.188           | 0.181            | 1.01          |
| br-C <sub>8</sub>  | 0.213           | 0.192            | 1.11          |
| br-C <sub>10</sub> | 0.188           | 0.184            | 1.02          |
| br-C <sub>12</sub> | 0.187           | 0.184            | 1.02          |
| TRIMETHYLOLETHANE  |                 |                  |               |
| n-C <sub>6</sub>   | 0.109           | 0.129            | 0.79          |
| n-C <sub>10</sub>  | 0.104           | 0.126            | 0.83          |
| br-C <sub>6</sub>  | 0.169           | 0.167            | 1.01          |
| br-C <sub>8</sub>  | 0.224           | 0.197            | 1.14          |
| br-C <sub>10</sub> | 0.184           | 0.181            | 1.02          |
| br-C <sub>12</sub> | 0.184           | 0.181            | 1.02          |
| TRIMETHYLOLPROPANE |                 |                  |               |
| n-C <sub>6</sub>   | 0.112           | 0.135            | 0.83          |
| n-C <sub>7</sub>   | 0.126           | 0.142            | 0.89          |
| n-C <sub>8</sub>   | 0.113           | 0.131            | 0.86          |
| n-C <sub>9</sub>   | 0.121           | 0.142            | 0.85          |
| n-C <sub>10</sub>  | 0.092           | 0.118            | 0.70          |
| br-C <sub>6</sub>  | 0.186           | 0.183            | 1.02          |
| br-C <sub>8</sub>  | 0.205           | 0.181            | 1.13          |
| br-C <sub>10</sub> | 0.181           | 0.177            | 1.02          |
| br-C <sub>12</sub> | 0.183           | 0.181            | 1.01          |
| PENTAERYTHRITOL    |                 |                  |               |
| n-C <sub>6</sub>   | 0.089           | 0.122            | 0.73          |
| br-C <sub>6</sub>  | 0.171           | 0.169            | 1.01          |
| br-C <sub>8</sub>  | 0.190           | 0.176            | 1.08          |
| br-C <sub>10</sub> | 0.174           | 0.172            | 1.01          |

| Acid                            | Static, $\mu_s$ | Kinetic, $\mu_k$ | $\mu_s/\mu_k$ |
|---------------------------------|-----------------|------------------|---------------|
| 2-BUTYL-2-ETHYL-1,3-PROPANEDIOL |                 |                  |               |
| n-C <sub>6</sub>                | 0.112           | 0.129            | 0.87          |
| n-C <sub>14</sub>               | 0.120           | 0.136            | 0.88          |
| n-C <sub>18</sub>               | 0.087           | 0.104            | 0.84          |

I have found that the esters of straight chain carboxylic acids and polyhydric alcohols free of beta hydrogens effectively increase the lubricity of silicone oils. The silicone oils are essentially polyorgano silicones (sometimes referred to as siloxanes) which may be represented by the general structure



where the R<sub>1</sub>, R<sub>2</sub> and R<sub>3</sub> is the same or a different hydrocarbon radical, such as straight or branched chain alkyl, aryl, alkaryl or aralkyl radicals and n is greater than 1. Examples of such radicals are methyl, ethyl, ethyl-methyl, phenyl, tolyl, phenyl-methyl, ethyl-phenyl, etc. The commercial silicone oils are essentially polymethyl siloxanes, polyethyl siloxanes and poly (methyl, phenyl) siloxanes. The molecular weights of silicone oils vary from about 200, for light oils to about 1,000 or more for the viscous oils.

The effectiveness of the herein-described esters of the present invention in improving the lubricity characteristics of silicone oils is illustrated by the data in Table III.

TABLE III

|    | Coefficient of Friction                                  |                  |               |      |
|----|----------------------------------------------------------|------------------|---------------|------|
|    | Static, $\mu_s$                                          | Kinetic, $\mu_k$ | $\mu_s/\mu_k$ |      |
| 45 | Silicone oil                                             | 0.299            | 0.294         | 1.02 |
|    | Silicone oil+10% trimethylolpropane-tri-n-nonoate        | 0.153            | 0.170         | 0.90 |
|    | Silicone oil+20% trimethylolpropane-tri-n-nonoate        | 0.141            | 0.160         | 0.87 |
| 50 | Silicone oil+10% neopentyl-di-n-nonoate                  | 0.160            | 0.174         | 0.92 |
|    | Silicone oil+20% neopentyl-di-n-nonoate                  | 0.150            | 0.161         | 0.93 |
|    | Silicone oil+20% neopentyl-di-br-nonoate                 | 0.225            | 0.223         | 1.01 |
|    | Diethyl adipate                                          | 0.262            | 0.174         | 1.51 |
|    | 20% trimethylolpropane-tri-n-nonoate+50% diethyl adipate | 0.206            | 0.195         | 1.06 |
| 55 | 50% trimethylolpropane-tri-n-nonoate+50% diethyl adipate | 0.196            | 0.194         | 1.01 |

The data in Table III demonstrate that as little as 10% of the esters of a polyhydric alcohol free of beta hydrogen and a straight chain carboxylic acid is effective in so improving the lubricity of silicone oils to give a smooth sliding lubricant, i.e. reduces the coefficient of friction value of  $\mu_s/\mu_k$  from 1.02 (sticking) to a value less than 1.00 (smooth sliding). However, the lubricity of other synthetic lubricating oils are not similarly affected. As shown by the data in Table III, the coefficient of friction value of  $\mu_s/\mu_k$  for diethyl adipate is not reduced to a value of 1 or less even by the addition of as much as 50% of trimethylolpropane-tri-n-nonoate.

The lubricant compositions of silicone oils and the esters of the present invention can, if desired, contain one or more other additives such as oxidation inhibitors, rust inhibitors, detergents, etc.

The percentages given herein are weight percentages unless otherwise stated.

I claim:

1. A lubricant composition comprising at least 25% of a silicone oil having the general structure



in which  $\text{R}_1$ ,  $\text{R}_2$  and  $\text{R}_3$  are radicals selected from the group consisting of methyl, ethyl, ethyl-methyl, phenyl, tolyl, phenyl-methyl, ethyl-phenyl radicals and mixtures thereof and from about 5% to about 75% of an ester of a straight chain aliphatic carboxylic acid of from about 4 to about 18 carbon atoms and a polyhydric alcohol free of beta-hydrogen, said ester having the general formula



in which  $\text{R}$  and  $\text{R}'$  are straight chain alkyl radicals having from 4 to about 18 carbons,  $\text{R}_1$  and  $\text{R}_4$  are constituents selected from the group consisting of hydrogen, alkyl radicals containing from 1 to 4 carbon atoms and mixtures thereof,  $\text{R}_2$  is a constituent selected from the group consisting of an alkyl radical having from 1 to 6 carbon atoms and a hydroxy methyl radical, and  $\text{R}_3$  is a constituent selected from the group consisting of an alkyl radical having from 2 to about 12 carbon atoms and a hydroxy methyl radical.

2. A lubricant composition comprising at least 25% of a silicone oil having the general structure



in which  $\text{R}_1$ ,  $\text{R}_2$  and  $\text{R}_3$  are radicals selected from the group consisting of methyl, ethyl, ethyl-methyl, phenyl, tolyl, phenyl-methyl, ethyl-phenyl radicals and mixtures thereof and from about 5% to about 75% trimethylol-propane-tri-n-nonoate.

3. A lubricant composition comprising at least 25% of a silicone oil having the general structure



in which  $\text{R}_1$ ,  $\text{R}_2$  and  $\text{R}_3$  are radicals selected from the group consisting of methyl, ethyl, ethyl-methyl, phenyl, tolyl, phenyl-methyl, ethyl-phenyl radicals and mixtures thereof and from about 5% to about 75% neopentyl-di-n-nonoate.

4. A lubricant composition comprising at least 25% of a silicone oil having the general structure



in which  $\text{R}_1$ ,  $\text{R}_2$  and  $\text{R}_3$  are radicals selected from the group consisting of methyl, ethyl, ethyl-methyl, phenyl, tolyl, phenyl-methyl, ethyl-phenyl radicals and mixtures thereof and from about 5% to about 75% trimethylol-ethane-tri-n-decanoate.

5. A lubricant composition comprising at least 25% of a silicone oil having the general structure



in which  $\text{R}_1$ ,  $\text{R}_2$  and  $\text{R}_3$  are radicals selected from the group consisting of methyl, ethyl, ethyl-methyl, phenyl, tolyl, phenyl-methyl, ethyl-phenyl radicals and mixtures thereof and from about 5% to about 75% 2-butyl-2-ethyl-1,3-propanediol-di-n-octadecanoate.

35 References Cited in the file of this patent

UNITED STATES PATENTS

|           |                |       |               |
|-----------|----------------|-------|---------------|
| 2,471,850 | Wilcock        | ----- | May 31, 1949  |
| 2,561,178 | Burkhard       | ----- | July 17, 1951 |
| 2,597,045 | Wilcock et al. | ----- | May 20, 1952  |
| 2,798,083 | Bell et al.    | ----- | July 2, 1957  |

FOREIGN PATENTS

|         |               |       |                |
|---------|---------------|-------|----------------|
| 715,933 | Great Britain | ----- | Sept. 22, 1954 |
|---------|---------------|-------|----------------|

UNITED STATES PATENT OFFICE  
CERTIFICATE OF CORRECTION

Patent No. 2,950,250

August 23, 1960

Morton Z. Fainman

It is hereby certified that error appears in the printed specification of the above numbered patent requiring correction and that the said Letters Patent should read as corrected below.

Column 2, line 58, Table I, first column thereof, for "br-C<sub>7</sub>" read -- br-C<sub>8</sub> --; column 3, lines 29 and 30, for "Lubrication Engineering" read -- Lubrication Engineering 2 --; column 5, lines 11 and 43, and column 6, lines 10, 21, and 33, after "thereof", each occurrence, insert -- and n is greater than 1 --.

Signed and sealed this 4th day of April 1961.

(SEAL)  
Attest: ERNEST W. SWIDER

XXXXXX  
Attesting Officer

ARTHUR W. CROCKER  
Acting Commissioner of Patents